# EUROPEAN PATENT APPLICATION

(11) **EP 1 447 474 A1**
(43) Date of publication of application: **18.08.2004**
(21) Application number: 04380015.0
(22) Date of filing: 21.01.2004
(51) Int. Cl.: D21H 21/44

(54) **Security paper**

(30) Priority: 11.02.2003 ES 200300329
(71) Applicant: Industrias de Hijos de Antonio Fabregas, S.A., 08301 Mataro (ES)
(72) Inventor: Margarit Daroca, Pedro, 08301 Mataro (ES)
(74) Representative: SUGRANES - VERDONCES - FERREGÜELA

(57) **Abstract**

Security paper which can be identified by the tearing thereof, which comprises a single base material or base sheet, coated on at least one of its sides, with one or several coloured layers, and an outer layer with opacifier properties which hide the middle coloured layers, which is suitable for printing with any printing means, the thickness of the security paper being less than 100 microns. The security paper can have a functional coating for thermal printing, either by thermal colour transference (thermal transference) or by melting of the micro-particles of which it is made (direct thermal).

## Description

### Technical field of the invention

The invention refers to security paper identified by the tearing thereof.

### Background of the invention

Authentication by tearing of a sheet of fibrous material, such as paper for example, consists of revealing by tearing an internal structure of multicoloured layers which are not visible from the outside without said tearing or ripping of the paper.

Papers which can be authenticated, also called security papers, identified by tearing, are very useful for producing documents such as entry tickets or travel tickets, paper money, legal documents, or any other document which may be exchangeable for a particular good or service.

Three types of structure for security paper identified by tearing are currently being used. The first consists in applying to coloured paper or card, a layer of white stucco on each side of the paper or card to cover the colour inside the card. This is a sandwich structure of white stucco coating/coloured material/white stucco coating.

The second structure used consists in a combination of three sheets joined together, of the type whose outside sheets are white and the middle one is coloured, producing a three-sheeted structure in which the coloured sheet is also sandwiched between the two outer sheets.

The third structure used consists in a combination of two joined sheets, one of which has at least one coloured side, whether this be with a layer of stucco, ink or dying glue which, when making the combination is positioned on the inside, being hidden by the other sheet.

Existing known security papers, which can be authenticated by tearing, have problems of delamination, which are inherent in multi-sheeted structures, as well as the fact that the minimum thickness of known security papers is greater than the thickness required for such applications, such as automatic validation in machines allowing exit or entry, in which the ticket to be validated has to be inserted or is issued through external slots which are generally flat and with a height limit of about 100 microns.

To solve the abovementioned problems, the security paper being the object of the invention fulfils the characteristics of being paper which is authenticated by tearing, which is not delaminable, cannot be falsified, is opaque, economical and which has good qualities in terms of printing and writing.

### Explanation of the invention

Security paper which is identified by the tearing thereof is, in essence, characterized in that it comprises a single base material or base sheet coated, on at least one of its sides, by one or several coloured layers, and an outer layer with opacifier properties which hide the middle coloured layers, the thickness of the security paper being less than 100 microns.

According to a preferred form of embodiment, the base material has, on one of its sides, a functional coating suitable for thermal printing, either by thermal colour transfer (thermal transfer) or by melting of the micro-particles of which it is made (direct thermal).

According to another aspect of the invention, the outer opacifier layer can be used for printing, whatever the printing means.

According to another characteristic of the invention, each of the coating layers, whether they are coloured, opacifier or functional, has a thickness of less than 16 microns.

### Brief description of the drawings

The attached drawings illustrate two non-limitative examples of forms of embodiment of security paper being the object of the invention. In said drawings:
Fig. 1, is a cross-section of the paper showing the base material and different layers of coating; and
Fig. 2, is a cross-section of a second form of embodiment of the security paper also showing the base material and different layers of coating.

### Detailed description of the drawings

The Security paper 1 being the object of the invention herein is made of a single base material 2 which can be of paper, card or any other synthetic material.

The lower side of the base material 2 in Fig. 1, is coated with a coloured layer 3 which, in turn, is coated with an opacifier layer 5 which hides, from the outside, the coloured layer 3, so that the latter is sandwiched between the base material 2 and the opacifier coating 5.

In the embodiment in Fig.2, however, there are two different coloured coatings 3 and 4 on the base material 2 and, as in the previous embodiment, there is an outer coating which hides the outer coloured layer 5. In reality, and due to the lack of thickness of the coloured layers, there can be as many different coloured layers as are needed between the base material 2 and the opacifier outer coating 5.

The opacifier coating 5 is usually made of components with a high reflection index (such as Titanium Dioxide TiO₂ components), or with products with lower reflection indexes, but with a very small particle size, which may be silicates, carbonates, kaolins, etc., the particle size being less than 2 microns.

To make the different coloured layers 3, 4, also called security layers, visible, invisible, photochromatic, iridescent, fluorescent, phosphorescent, chemically or heat-reactible, etc. colorants can be used, on all or each of the coloured layers of the security paper.

As for the base material 2 to which the coloured layers 3, 4, are applied, these can be offset paper or card (without surface coating) or, otherwise, can be surface coated 6, as shown in Figs. 1 and 2, which can be white or coloured stucco, a treated coating suitable for printing by thermal transference or thermal transfer (a toner or strip melts under heat and is transferred to the coating by adhering to it) or by direct thermal type (heat is applied to the coating and the micro particles it is made of, upon melting, release the colour).

In all cases, to check the authenticity of the paper, such as the one in the invention, all that has to be done is tear the paper to see from the outside the coloured layer or layers 3, 4 which are hidden on the inside of the paper 1.

As the different layers covering the base material 2 have a thickness of approximately 20 microns, security papers which can be easily authenticated, with a thickness of less than 100 microns, can be obtained. Currently known security papers, which use the tearing method, are made up of more than one sheet or base material, which means that the thickness that can be obtained is always more than 100 microns.

### Examples of embodiment

A single Termotag CT fibrous base material of 80 microns is used, manufactured by Fábregas (Mataró), or a 150 UTB quality base material of 80 microns, manufactured by Ricoh (Japan), both already provided with a functional layer on each side which allows printing via the "direct thermal" system, and on the reverse side (the opposite side to the one to be thermally printed) has the following layers:
- One or more layers coloured with light-visible pigments, with a thickness of between 10 and 20 microns. These coloured layers, which can be dispersed in water or solvents, are made up of:
   A) Pigments: 5% to 95% in weight are pigments coloured with the relevant colour, for example green, and the remaining 95% to 5% are mineral elements (calcium sulphate, calcium carbonate, kaolin, talc, dolomites, silicates of the type used for elements in paints or paper stuccos).
   B) Binders: 7% to 50% in weight of the pigments. It is preferable that the pigments be adhered together and to the base material. Casein, latex can be used: butadiene styrene, acrylics, polyvinyl acetates, vinyl acetate copolymers, acrylic resin copolymers, styrene resin copolymers, starches, starch ethers, carboxymethycelluloses, polyvinyl alcohols, nitrocellulose resins, maleic ethers or any other chemical component suitable for adhering.
   C) Extension and film-forming enhancers: These are present in a proportion comprising between 0.05% and 0.5% of the pigments. Formed by anti-foaming agents, silicones, stearates, various surface-active agents, sulfosuccinates or polyalcohols.
- An outer opacifier layer, with a thickness of between 10 and 20 microns, white in colour for example, suitable for printing with any traditional printing system (offset, photogravure, flexographic, transfer, silk screen), which hides the coloured layer. Said opacifier layer can be dispersed in water or with solvents and is made up of:
   A) Pigments: 5% to 95% are high-opacity pigments, such as titanic dioxide, silicates, colloidal silica, kaolin or calcium carbonate. The remaining 95% to 5% are mineral elements (calcium sulphate, calcium carbonate, kaolin, talc, dolomites, silicates of the type used as elements in paints or paper stuccos).
   B) Binders: 7% to 50% in weight of the pigments. It is preferable that the pigments be adhered together and to the base material. Casein, latex can be used: butadiene styrene, acrylics, polyvinyl acetates, vinyl acetate copolymers, acrylic resin copolymers, styrene resin copolymers, starches, starch ethers, carboxymethycelluloses, polyvinyl alcohols, nitrocellulose resins, maleic ethers or any other chemical component suitable for adhering.
   C) Extension and film-forming enhancers: These are present in a proportion comprising between 0.05% and 0.5% of the pigments. Formed by anti-foaming agents, silicones, stearates, various surface-active agents, sulfosuccinates or polyalcohols.

Once the paper is coated with the layers described above, it is calendered until the required micron level is obtained.

Paper without the functional layer 5 can quite easily be used, to which the security treatment of the invention is applied.

## Claims

1. Security paper (1) which can be identified by the tearing thereof, **characterized in that** it comprises a single base material (2) or base sheet, coated on at least one of its sides, by one or several coloured layers (3, 4), and an outer layer (5) with opacifier properties which hide the middle coloured layers (3, 4), the thickness of the security paper (1) being less than 100 microns.

2. Paper according to claim 1, **characterized in that** the base material (2) has, on one of its sides, a functional coating (6) suitable for thermal printing, either by thermal colour transference (thermal transference) or by melting of the micro-particles of which it is made (direct thermal).

3. Paper according to claims 1 or 2, **characterized in that** the outer opacifier layer (5) can be used for printing, whatever the printing means. '

4. Paper according to the previous claims, **characterized in that** each of the coating layers, whether they are coloured (3, 4), opacifier (5) or functional (6), has a thickness of less than 20 microns.
